

# UNITED STATES PATENT OFFICE.

FRANÇOIS RIBBE, OF MAURIAC, AND PAUL DHÉ, OF PARIS, FRANCE.

## PROCESS FOR THE CONSTRUCTION OF MONOLITHIC STRUCTURES OF BASALT.

1,331,377.

Specification of Letters Patent.

Patented Feb. 17, 1920.

No Drawing.

Application filed November 5, 1918. Serial No. 261,313.

To all whom it may concern:

Be it known that we, FRANÇOIS RIBBE, of No. 26 Avenue de la Gare, Mauriac, Cantal, France, doctor of medicine, and PAUL DHÉ of No. 42 ter Rue Notre Dame des Champs, Paris, France, engineer, and citizens of the Republic of France, have invented certain new and useful Improved Processes for the Construction of Monolithic Structures of Basalt, of which the following is a specification.

The French Patent No. 449707 applied for on 29 December 1911 contains a description of methods of casting, molding and 15 vitrifying on the actual surface of the ground, various articles of basalt that has been previously melted in cupola furnaces mounted on a carriage. The invention described in the said patent has more particularly for its object the manufacture of slabs 20 intended to serve as a protective covering for roads.

The present invention has for its object to produce, likewise, at the place of their future use and also by melting, molding and devitrifying processes, various structures, composed of basalt or other volcanic rock, more often in one piece and of considerable dimensions, such as dams, sea-walls, piers, 30 bridges, fortifications etc.

Hereinafter a description is given by way of example, of the manner of constructing a dam for damming a stream.

The shape of the structure has nothing 35 peculiar in it. Nevertheless in general it is advisable to arrange that the basalt shall act in compression. The structure will therefore be given a certain amount of curvature with its convex side facing up- 40 stream of course.

The ground after having been excavated down to the solid stratum according to the adopted plan and in accordance with the rules of the art, is then dried as far as it 45 is possible. If any moisture remains, a very light layer of basalt ballast will prevent any excessive formation of air bubbles. The casting operations may then begin.

The furnaces may be fixed or portable. 50 In the former case they should be erected at the most convenient points in the immediate neighborhood of the structure to be built. They may be of widely varying types; in some cases it may be best to employ 55 an electric furnace. Generally however, it is preferred to use a cupola furnace, when

the dam to be built is of large size, and it is not feared to change the chemical composition of the material within certain limits, it will be an advantage to choose apparatus of 60 the blast furnace type.

These allow of a much better utilization of the heat, and by the reduction of a part of the iron oxids of the basalt, they produce a certain amount of iron that can be sold at 65 a fairish price.

The molten basalt is to be convoyed to the points where it is to be cast, by means of portable fore-hearths, ladles or other suitable vessels adapted to travel on aerial cable 70 ways or on rails supported on scaffolds on each side of the work.

Portable furnaces, where their use is necessitated by exceptional circumstances will be mounted on balls or on wheels and will 75 be adapted to travel along the rails on the scaffolds.

In a case where the width of the dam should render it necessary, the said furnaces would be located on traveling bridges provided with rails extending right across the dam, these traveling bridges being in their turn adapted to travel on the rails of the scaffolds. In this manner and owing to the two-fold mobility of the furnaces along the 85 traveling bridges, and of the traveling bridges along the entire structure, there is no point of the dam that cannot be reached by the casting operation. The apparatuses are charged by means of aerial cable ways or 90 any other suitable means.

It is to be understood that a plurality of furnaces may be arranged to travel simultaneously, and that arrangements are made for removing and replacing any of the 95 apparatus that may require repair.

It is also to be understood that the traveling bridges may be used in certain cases for the conveyance of ladles charged with material that has been melted in fixed 100 furnaces.

But whatever may be the system of melting and conveyance that is adopted, it will be necessary, except in rare cases, to employ only a "non-bubbly" material, which on 105 cooling will form a dense rock of great strength. This condition is easily satisfied by basalt which in the state of liquid fusion, allows of a rapid escape of its bubbles in the vessels in which it is received as it is 110 run from the furnaces.

The shape to be given to the dam is pro-

duced in a very simple manner. So long as the work is being built up in the excavation, the sides of the latter will serve as the mold. On leaving the excavation the fluid material is contained at suitable points by a line of frames set side by side lined with bricks which may be porous or non-porous, but are well "talced" or rubbed with cinder if it is desired to prevent adhesion. The frames are allowed to remain in place for a certain number of days so as to prevent the sides of the structure from cooling too quickly, after which they may be removed for re-use.

Instead of bricks, there may be employed slabs of baked earth, cast iron, or plates of very dry cement or other means. In some cases where there is no objection to having sides of very irregular shape and with a slope, molding may be dispensed with altogether.

These preliminary arrangements having been made, the following is a description of the manner of making the block, and how it is possible by means of daily castings to produce a monolithic structure constituting a real natural rock having enormous strength of resistance.

When a casting of molten basalt has not great thickness, the material soon solidifies, but if while it is still hot, although its temperature has fallen to below red heat, a fresh casting is poured upon its surface, its more superficial parts will become melted again and an intimate union will be produced between the two masses. Consequently as the dam increases in height, the quantity of material that is added every day to its surface will become united by autogenous welding to the underlying block and will form absolutely one piece therewith. Moreover it will serve to complete the devitrification of those portions of the mass of the preceding casting which by having cooled too quickly, may have acquired a vitreous character.

One condition however which must be considered as being almost essential to success, is this, namely, the work of constructing the dam when once begun, must never be interrupted, in other words a sufficient quantity of material must be poured upon each point of the surface of the monolithic structure before the temperature at that point has fallen too close to the temperature of the atmosphere. Consequently every care must be taken in every respect to assure that the dam shall receive each day on its surface so much fresh material as will raise the height of the dam by at least some decimeters approximately uniformly throughout its extent.

Therefore unless the daily addition of material is great, it is necessary at least to provide some protection against a rapid cooling of the liquid basalt that is being continually

poured upon the dam in course of construction. Such protection is necessary in order that the autogenous welding shall hold. Such protection is further necessary to assure the devitrification of the material whereby the rock regains all its resisting power. For this purpose a layer of hot and relatively stagnant air is formed at its surface by means which may vary considerably.

Among such means, there is one which has proved its efficiency, namely the arrangement of frames lined with porous bricks supported by their ends directly upon the scaffolds when the width of the work is not too great, or resting on stretched ropes or on a metal framework provided for this purpose in other cases, but always arranged side by side in such a manner as to form a continuous horizontal screen for a small height above the surface of the basalt. When a casting operation has to be done at any point, the corresponding frame will be temporarily moved aside.

If by reason of untoward circumstances the work has been discontinued for so long a time as to cause a complete cooling of its surface, it will be necessary to resume the pourings in the ordinary way, and then some hours afterward to break up the product of the pouring at all places where a sufficient welding has not been effected with the preceding casting. The old surface having thus been well reheated, will then be more adapted to make a good weld with the fresh molten masses with which it will be presently covered.

Or the cooled surface may be covered with a thin layer of cement or a layer of bricks cemented together upon which, after the same has become dry, the pourings are resumed.

In most cases it will be advantageous to employ reinforced basalt instead of ordinary basalt. The resisting power of the block will be greatly increased thereby, while in the case of an interruption of the construction the resumption of the work will also be facilitated.

With a view to economy, there may be introduced into the molten material either before or after the casting *in situ*, a certain quantity of basalt, granite, flint or other rocks that will not be liable to become decomposed by the temperature of the bath, such rocks should be coarsely crushed. These fragments will unite to form one piece with the basalt on the cooling of the latter. In order to prevent the inconvenient formation of bubbles, only lumps should be used which have first been freed by suitable heating from their natural water content and the greater portion of their occluded gases, and they are mixed with the basalt while they are still hot.

As soon as the monolithic block has

reached a certain height it may be called upon to support its own scaffolding. For this purpose pieces of iron in suitable number and of suitable strength are inserted in 5 the block; holes and recessed or projecting parts are formed at suitable points; all for the purpose of providing supports for the scaffolds at the sides. The stepped sloping side of the actual dam may even be utilized 10 for this purpose.

It is scarcely necessary to mention any of the advantages afforded by the use of monolithic basalt structures. The enormous strength of this material will allow of reducing appreciably the total cubic content 15 of such structures compared with the cubic content of the ordinary masonry or brick-work which it replaces, while increasing however the margin of safety. No upkeep, 20 and practically no watching are required.

The improved method allows of building bridges, viaducts, various works of fortification such as parapets, escarpment and counter-escarpment walls, open caponieres, 25 aprons for armor, emplacements for large guns, and even casemates because basalt, especially when reinforced, is very suitable for the construction of roofs or vaultings. It may also be employed in the construction 30 of wall foundations, and also entire walls, even for dwellings, which, in addition to their unshakable firmness, have the advantage of being capable of very rich ornamentation. This enumeration has no limiting force whatever, because any structures 35 of the kind hereinbefore referred to, can be constructed of the same material and by the same method, barring slight modifications according to the circumstances of each case.

40 Having now particularly described and ascertained the nature of our said invention, and in what manner the same is to be per-

formed we declare that what we claim is:—

1. A method of constructing constructional works, dams, barrages, fortifications, 45 bridges and the like structures, which consists in casting molten basalt in successive superposed layers in the actual space which the desired structure is to occupy, each new layer being cast while the preceding layer 50 is still sufficiently hot to become welded to the said new layer, whereby the whole forms a monolithic structure.

2. A method of constructing constructional works, dams, barrages, fortifications, 55 bridges and the like structures, which consists in casting molten basalt in successive superposed layers in the actual space which the desired structure is to occupy, the cooling of the top surface of the structure as 60 it is being built, being reduced by means of a screen which placed upon it and which retains a layer of air on the cast basalt.

3. A method of constructing constructional works, dams and the like structures, 65 which consists in casting molten basalt in successive superposed layers in the actual space to be occupied by the desired structure, and incorporating, heated stones successively into the layers of basalt while the 70 said layers are still fluid.

4. A method of constructing constructional works, dams, and the like structures, which consists in casting molten basalt in successive superposed layers in the actual 75 space to be occupied by the desired structure, from casting appliances that are adapted to travel on scaffolds which rest on the actual structure and which are raised according as the said structure increases in 20 height.

FRANÇOIS RIBBE.  
PAUL DHÉ.